

## UNITED STATES PATENT OFFICE

CHARLES G. CHEVALIER, OF BALTIMORE, MARYLAND

## COMPOUND FOR CLEANING

No Drawing.

Application filed May 5, 1928. Serial No. 275,562.

My invention relates to a method and compound for cleaning, and particularly to one especially adapted for the removal of all oil, grease, or the like adhering to sheets of new 5 tinplate, or other rolled sheet metal.

In the processes used for manufacturing tinplate, the finished sheets generally have a thin film of oil adhering thereto. Such a film prevents successful soldering operations 10 on articles made from such oily sheets, and also prevents a perfect coating or printed impressions being made on such articles.

One method used for cleaning oily sheets has been to place such sheets in a machine 15 containing a batch of the coarser part of ground wheat which is generally called "middlings". At first this works fairly well, but after about twenty minutes these middlings lose their cleaning power, with the 20 result that if the process is continued longer the sheets come out with a thin film of oil or grease still adhering thereto. Many shipments are returned to the manufacturers for re-cleaning, because of such films.

25 With the machine formerly used each renewal of the middlings requires the stopping of the machine, the removal of the old exhausted batch and its replacement with a fresh batch. Such frequent renewals are obviously 30 objectionable and increase the cost of cleaning.

A new type of cleaning machine has been perfected which permits the replacement of an exhausted batch with a fresh one, without 35 stopping the machine.

I have discovered that with the addition of a small amount of powdered diatomaceous earth, a new result is obtained. With my compound the interval between renewals of 40 the middlings may be increased from twenty minutes to five hours, or about fifteen times, with satisfactory results. The action of this small amount of earth seems to be to scrape the oil film from the plate, and that when so 45 removed this oil is much more readily absorbed by the middlings. The amount of this diatomaceous earth which I have found to give satisfactory results is from one percent to five percent, by weight, to each batch 50 of middlings.

Diatomaceous earth also has a capacity for absorbing oil and grease, and, if desired, larger proportions of it may be used in my compound.

With my compound the tinplate sheet may 55 be freed entirely from oil or grease, leaving the surface in the proper condition for subsequent soldering or decorating of articles made therefrom. With the advantage of this more perfect cleaning and polishing of the 60 sheets, there is obviously a great saving in the cost over using middlings alone.

The cost of my process is further reduced 65 because after the middlings and powdered diatomaceous earth have taken up all the oil which the compound is capable of removing satisfactorily, it may be sold as a cattle feed 70 as "palmo-middlings".

Various modifications of my invention 75 within the scope of the claims may be made, for instance the method may be used to clean articles which are not in the shape of sheets, and to remove any other coating which the middlings are capable of absorbing.

Neither the earth, middlings or oil can be 80 readily separated or recovered and used again, and in view of the market for this cattle feed, there seems to be no need for doing so.

Varying conditions such as the smoothness 85 of the rolled sheets upon which the tin coating is formed, the quality and temperature of the oil, make it necessary to vary the period of use of my compound to meet such conditions.

## What I claim is:

1. An oil removing and surface polishing compound consisting of a finely divided oil absorbent material to which has been added diatomaceous earth. 90

2. An oil removing and surface polishing compound consisting of middlings to which from one to five percent of diatomaceous earth has been added. 95

3. An oil removing and surface polishing compound consisting of middlings and diatomaceous earth. 100

In testimony whereof I hereunto affix my signature.

CHARLES G. CHEVALIER. 100